

1

3,082,088

## PROCESS FOR MAINTAINING THE CLARITY OF PHOTOGRAPHIC SILVER HALIDE EMULSIONS AT RELATIVELY HIGH DEVELOPER TEMPERATURES

Max Heilmann, Kohn-Flittard, and Wilhelm Jessien and Werner Stracke, Leverkusen, Germany, assignors to Agfa Aktiengesellschaft, Leverkusen, Germany, a corporation of Germany

No Drawing. Filed Jan. 11, 1961, Ser. No. 81,949

Claims priority, application Germany Jan. 16, 1960

4 Claims. (Cl. 96—109)

The invention is concerned with a process for improving the clarity of photographic silver halide emulsions during development at relatively high temperatures.

Photographic silver halide emulsions have a tendency at relatively high developer temperatures to give a considerable degree of fogging which appreciably impairs the quality of the picture. Since relatively high developer temperatures frequently cannot be avoided, because of unfavorable climatic conditions, it has long been desired to prevent the formation of this development fog by adding suitable substances to the photographic silver halide emulsion, to the photographic auxiliary layers, or to the processing baths.

A number of substances have also been described which have the effect of keeping the unexposed silver halide clear, but these influence disadvantageously other photographic properties in one way or another. The most important of these substances include benztriazole, which substantially prevents fog formation, but simultaneously shifts the tone of the image undesirably towards blue-black. The use of urea and its substitution products as fog inhibitors is described in U.S. Patent No. 1,763,990. However, these fog inhibitors are not able to prevent the development of fog which occurs at relatively high developer temperatures.

It has now been found that the fog formation at relatively high developer temperatures can largely be prevented if, to the photographic silver halide emulsion or photographic auxiliary layers, such as protective or intermediate layers or the like, are added, prior to the casting, substituted 4(5)-aminobenztriazoles of the following general formula:



in which R represents an aliphatic radical with at least two carbon atoms, an aromatic or heterocyclic radical which in turn may be substituted, and X represents a simple chemical bond, an oxygen atom or an imino radical and in which the benzene nucleus may also carry other substituents.

Suitable substances for this purpose that conform to the foregoing formula are acylated aminobenztriazoles, such as 5-benzoylaminobenztriazole, carbamic acid derivatives such as 5-carbethoxyaminobenztriazole, 5-carbo-phenoxyaminobenztriazole, 4-carbo-phenoxyaminobenztriazole, 4-carbo-phenoxyamino-6-aminobenztriazole and urea derivatives of benztriazole, such as N-ethyl-N'-(5)-benztriazolyl urea, N-phenyl-N'-(4)-benztriazolyl urea, N-phenyl-N'-(5)-benztriazolyl urea, N-(4'-ethoxyphenyl)-N'-(5)-benztriazolyl urea, N-(3'-chlorphenyl)-N'-(5)-benztriazolyl urea, N-(4'-chlorphenyl)-N'-(5)-benztriazolyl urea.

The preparation of these compounds may be effected by known methods.

The acylated aminobenztriazoles are obtained by reac-

2

tion of equivalent quantities of an aminobenztriazole with an acid chloride in the presence of an acid-binding agent, such as pyridine.

The carbamic acid derivatives are obtained by reacting a chloroformic acid ester with an aminobenztriazole.

The urea derivatives are obtained by reaction with isocyanates. This reaction can take place without solvents or in suspension in an inert solvent or in a tertiary nitrogen atom-containing solvent. Benztriazole urea derivatives substituted by heterocyclic radicals are prepared, for example, by reaction of cyclotetramethylenesulfonisocyanate with 4- or 5-aminobenztriazole. There are thus obtained substances of the following formula:



The outstanding efficacy of the substances according to the invention is apparent from the following table, which reproduces the fog values of a silver bromide emulsion according to Bios Final Report No. 252, which emulsion had been cast with and without addition of aminobenztriazole derivatives, after development for 4 minutes at 30° C.

|                                                    | Fog density<br>after develop-<br>ment at 30° C. |
|----------------------------------------------------|-------------------------------------------------|
| Silver bromide emulsion:                           |                                                 |
| Without additive                                   | 0.052                                           |
| With N-ethyl-N'-(5)-benztriazolyl urea (Example 2) | 0.031                                           |
| With N-phenyl-N'-(4)-benztriazolyl urea 1          | 0.009                                           |
| With N-phenyl-N'-(5)-benztriazolyl urea            | 0.015                                           |
| With N-(4'-ethoxyphenyl)-N'-(5)-benztriazolyl urea | 0.015                                           |
| With N-(3'-chlorphenyl)-N'-(5)-benztriazolyl urea  | 0.017                                           |
| With N-(4'-chlorphenyl)-N'-(5)-benztriazolyl urea  | 0.009                                           |
| With 5-benzoylaminobenztriazole (Example 1)        | 0.038                                           |
| With 5-carbo-phenoxyaminobenztriazole              | 0.017                                           |
| With 4-carbo-phenoxyaminobenztriazole              | 0.033                                           |
| With 4-carbo-phenoxyamino-6-aminobenztriazole      | 0.027                                           |
| With 4-benzoylaminobenztriazole                    | 0.041                                           |
| With 5-carboethoxyaminobenztriazole                | 0.037                                           |

1 This compound is also referred to as 4-(3-phenyl-ureido)-1,2,3-benzotriazole.

If N-phenyl-N'-(5)-benztriazolyl urea is added to a protective layer, the fog value after development for 4 minutes at 30° C. is 0.045, whereas the fog value without adding the stabilizer increases to 0.195. The emulsion used for this test was the same as mentioned above but this batch was very susceptible to fog formation.

The substances according to the invention may be used in quantities from 5 to 250 mg. per liter of emulsion. 1 liter of emulsion contains approximately 30 g. of silver halide.

The substances according to the invention are suitable for reducing the fogging of silver chloride, silver bromochloride and silver bromide emulsions, and the maximum effect is produced with silver bromide-ammonia emulsions. The emulsions may contain up to 5 percent silver iodide.

### Example 1

A silver bromide emulsion containing 110 g. of AgBr to

3

5 liters has added thereto 8 cc. per liter of a 1% solution of the compound



After adding the other conventional hardening agents, the emulsion is cast on to paper.

The fog value with and without addition of stabilizer, after 4 minutes development at 30° C., are set out in the foregoing table. Development is carried out in a conventional metol-hydroquinone developer which is made alkaline with soda.

*Example 2*

A silver bromochloride emulsion containing about 35 g. of AgBr and 70 g. of AgCl to three liters has added thereto, 3 cc. per liter of a 1 percent solution of the compound:



and the emulsion is cast after addition of other hardening agents.

When the stabilizer is added the fog value after development for 4 minutes is 0.015 whereas it is 0.124 when no stabilizer has been added.

*Example 3*

The stabilizer of the formula



was prepared as follows:

4 grams of 5-aminobenztriazole and 5.2 grams of the hydrochloride of isonicotinic acid chloride are refluxed for 3 hours in 50 cm.<sup>3</sup> of pyridine. The reaction mixture was precipitated by addition of water, filtered and recrystallized from dimethylformamide. The product melts at 338° C. under decomposition.

50 mg. of the above-mentioned compound were added to 1 liter of a silver bromide emulsion according to Bios Final Report No. 252. The development is achieved in the conventional metol-hydroquinone developer which is made alkaline with soda. After 4 minutes developing at 30° C. the fog value without addition of stabilizer was 0.141 while in the presence of the above-mentioned stabilizer the fog value was only 0.117. The batch of the above-mentioned silver bromide emulsion was very susceptible to fog formation.

*Example 4*

The stabilizer of the formula



was prepared as described in Example 3 except that 4-aminobenztriazol was used as starting compound. Development was accomplished as described in the foregoing example. After 4 minutes developing at 30° C. the fog

value without addition of stabilizer was 0.113 while in the presence of the stabilizer of the above-mentioned formula the fog value was only 0.076.

4

*Example 5*

The stabilizer of the formula



was prepared by reaction of cyclo-tetra-methylene sulfone-isocyanate with 5 amino-benztriazole. Development was carried out as described in Example 4. The fog value without addition of the stabilizer was 0.113. The fog value was reduced by this stabilizer to 0.06.

It is to be understood that the stabilizers according to the invention may be substituted by various groups, for example the following compounds are suitable stabilizers:



prepared by reaction of butyrolactone with 5-amino-benztriazole;



prepared by reaction of a chloro-substituted fatty acid ester with 5-amino-benztriazole;



45 prepared by reaction of acetoacetic ester with 5-amino-benztriazole;



prepared by reaction of hexamethylene diisocyanate with 5-amino-benztriazole;



prepared by reaction of a chloro-substituted alkylene isocyanate with 5-amino-benztriazole;



70 prepared by reaction of alphanaphthyl isocyanate with 5-amino-benztriazole.

What is claimed is:

75 1. A photographic material which comprises a light-

sensitive silver halide emulsion layer and a contiguous auxiliary layer, at least one of which layers contains a derivative of amino-benztriazole selected from those having the following general formulae:



in which R represents a radical selected from the class consisting of alkyl with at least 2 carbon atoms, substituted alkyl with at least 2 carbon atoms, aryl, substituted aryl, heterocyclics and substituted heterocyclics; X

being a member selected from the group consisting of a simple chemical bond, an oxygen atom, and an imine radical, in an amount sufficient to inhibit the formation of fog in the subsequent development of the silver halide emulsion layer of the said photographic material at a relatively high development temperature.

- 5 2. A photographic material as defined in claim 1, the light-sensitive silver halide emulsion layer of which contains an aminobenztriazole derivative as defined in claim 1.
- 10 3. The photographic material as defined in claim 1 the contiguous photographic auxiliary layer of which contains the amino-benztriazole derivative as defined in claim 1.
- 15 4. A photographic material as defined in claim 1, the silver halide emulsion layer of which contains 4-(3-phenylureido)-1,2,3-benzotriazole.

References Cited in the file of this patent

FOREIGN PATENTS

20 350,996 Great Britain ----- June 19, 1931